



US006033623A

# United States Patent [19]

Deevi et al.

[11] Patent Number: 6,033,623

[45] Date of Patent: Mar. 7, 2000

[54] **METHOD OF MANUFACTURING IRON ALUMINIDE BY THERMOMECHANICAL PROCESSING OF ELEMENTAL POWDERS**

[75] Inventors: **Seetharama C. Deevi**, Midlothian; **A. Clifton Lilly, Jr.**, Chesterfield, both of Va.; **Vinod K. Sikka**, Oak Ridge, Tenn.; **Mohammed R. Hajaligol**, Richmond, Va.

[73] Assignee: **Philip Morris Incorporated**, New York, N.Y.

[21] Appl. No.: **08/679,341**

[22] Filed: **Jul. 11, 1996**

[51] Int. Cl.<sup>7</sup> ..... **B22F 3/18**; B22F 3/24

[52] U.S. Cl. ..... **419/45**; 419/29; 419/43; 419/36

[58] Field of Search ..... 419/26, 2, 28, 419/43, 45, 53, 54, 29, 36

[56] **References Cited**

## U.S. PATENT DOCUMENTS

|           |         |                   |
|-----------|---------|-------------------|
| 1,550,508 | 8/1925  | Cooper .          |
| 1,990,650 | 2/1935  | Jaeger .          |
| 2,768,915 | 10/1956 | Nachman et al. .  |
| 3,026,197 | 3/1962  | Schramm .         |
| 3,676,109 | 7/1972  | Cooper .          |
| 4,334,923 | 6/1982  | Sherman .         |
| 4,391,634 | 7/1983  | Kelly et al. .    |
| 4,684,505 | 8/1987  | Brinegar et al. . |
| 4,961,903 | 10/1990 | McKamey et al. .  |
| 5,024,109 | 6/1991  | Romero et al. .   |
| 5,032,190 | 7/1991  | Suarez et al. .   |
| 5,084,109 | 1/1992  | Sikka .           |
| 5,158,744 | 10/1992 | Nazmy .           |
| 5,238,645 | 8/1993  | Sikka et al. .    |
| 5,249,586 | 10/1993 | Morgan et al. .   |
| 5,320,802 | 6/1994  | Liu et al. .      |

## FOREIGN PATENT DOCUMENTS

|        |        |          |
|--------|--------|----------|
| 648140 | 9/1962 | Canada . |
| 648141 | 9/1962 | Canada . |

53-119721 10/1978 Japan .

## OTHER PUBLICATIONS

J.R. Knibloe et al., Advances in Powder Metallurgy, vol. 2, "Microstructure And Mechanical Properties of P/M Fe<sub>3</sub>Al Alloys", (1990) pp. 219-231.

V.K. Sikka, Mat. Res. Soc. Symp. Proc., vol. 213, "Powder Processing of Fe<sub>3</sub>Al-Based Iron-Aluminide Alloys," (1991) pp. 901-906.

V.K. Sikka et al., "Powder Production, Processing, and Properties of Fe<sub>3</sub>Al", pp. 1-11, presented at the 1990 Powder Metallurgy Conference Exhibition in Pittsburgh, PA.

(List continued on next page.)

Primary Examiner—Daniel J. Jenkins  
Attorney, Agent, or Firm—Burns, Doane, Swecker & Mathis, L.L.P.

[57] **ABSTRACT**

A powder metallurgical process of preparing iron aluminide useful as electrical resistance heating elements having improved room temperature ductility, electrical resistivity, cyclic fatigue resistance, high temperature oxidation resistance, low and high temperature strength, and/or resistance to high temperature sagging. The iron aluminide has an entirely ferritic microstructure which is free of austenite and can include, in weight %, 20 to 32% Al, and optional additions such as  $\leq 1\%$  Cr,  $\geq 0.5\%$  Zr or ZrO<sub>2</sub> stringers extending perpendicular to an exposed surface of the heating element,  $\leq 2\%$  Ti,  $\leq 2\%$  Mo,  $\leq 1\%$  Zr,  $\leq 1\%$  C,  $\leq 0.1\%$  B,  $\leq 30\%$  oxide dispersoid and/or electrically insulating or electrically conductive covalent ceramic particles,  $\leq 1\%$  rare earth metal,  $\leq 1\%$  oxygen, and/or  $\leq 3\%$  Cu. The process includes forming a mixture of aluminum powder and iron powder, shaping the mixture into an article such as by cold rolling the mixture into a sheet, and sintering the article at a temperature sufficient to react the iron and aluminum powders and form iron aluminide. The sintering can be followed by hot or cold rolling to reduce porosity created during the sintering step and optional annealing steps in a vacuum or inert atmosphere.

25 Claims, 21 Drawing Sheets



## OTHER PUBLICATIONS

- A. LeFort et al., "Mechanical Behavior of  $\text{FeAl}_{40}$  Intermetallic Alloys" presented at the Proceedings of International Symposium on Intermetallic Compounds—Structure and Mechanical Properties (JIMIS-6), pp. 579–583, held in Sendai, Japan on Jun. 17–20, 1991.
- D. Poccia et al. "Production and Properties of CSM FeAl Intermetallic Alloys" presented at the Minerals, Metals and Materials Society Conference (1994 TMS Conference) on "Processing, Properties and Applications of Iron Aluminides", pp. 19–30, held in San Francisco, California on Feb. 27—Mar. 3, 1994.
- J. H. Schneibel, "Selected Properties of Iron Aluminides", pp. 329–341, presented at the 1994 TMS Conference.
- J. Baker, "Flow and Fracture of FeAl", pp. 101–115, presented at the 1994 TMS Conference.
- D.J. Alexander, "Impact Behavior of FeAl Alloy FA-350", pp. 193–202, presented at the 1994 TMS Conference.
- C.H. Kong, "The Effect of Ternary Additions on the Vacancy Hardening and Defect Structure of FeAl", pp. 231–239, presented at the 1994 TMS Conference.
- D. J. Gaydosh et al., "Microstructure and Tensile Properties of Fe-40 At.Pct. Al Alloys with C, Zr, Hf and B Additions" in the Sep. 1989 Met. Trans A, vol. 20A, pp. 1701–1714.
- C. G. McKamey et al., "A review of recent developments in  $\text{Fe}_3\text{Al}$ -based Alloys" in the Aug. 1991 J. of Mater. Res., vol. 6, No. 8, pp. 1779–1805.



FIG. 1A



FIG. 1B



FIG. 1C



FIG. 1D



FIG. 2A



FIG. 2B



**FIG. 3A**



FIG. 3B



FIG. 4A



FIG. 4B



FIG. 5A



FIG. 5B



FIG. 6A



FIG. 6B



FIG. 7



FIG. 8A



FIG. 8B



FIG. 8C

**FIG. 9A****FIG. 9B****FIG. 9C**



FIG. 10A



FIG. 10B



FIG. 10C



FIG. 10D



FIG. 11A



FIG. 11B



FIG. 12A



FIG. 12B



FIG. 12C



FIG. 12D



FIG. 12E



FIG. 13A



FIG. 13B



FIG. 13C



FIG. 14A



FIG. 14B



FIG. 14C



FIG. 14D



FIG. 14E



FIG. 15A



FIG. 15B



FIG. 16A



FIG. 16B

## METHOD OF MANUFACTURING IRON ALUMINIDE BY THERMOMECHANICAL PROCESSING OF ELEMENTAL POWDERS

### STATEMENT OF GOVERNMENT RIGHTS

The United States government has rights in this invention pursuant to contract no. DE-AC05-840R21400 between the United States Department of Energy and Lockheed Martin Energy Research Corporation, Inc.

### FIELD OF THE INVENTION

The invention relates generally to iron aluminide and a powder metallurgical technique for preparation of such materials.

### BACKGROUND OF THE INVENTION

Iron base alloys containing aluminum can have ordered and disordered body centered crystal structures. For instance, iron aluminide alloys having intermetallic alloy compositions contain iron and aluminum in various atomic proportions such as  $Fe_3Al$ ,  $FeAl$ ,  $FeAl_2$ ,  $FeAl_3$ , and  $Fe_2Al_5$ .  $Fe_3Al$  intermetallic iron aluminides having a body centered cubic ordered crystal structure are disclosed in U.S. Pat. Nos. 5,320,802; 5,158,744; 5,024,109; and 4,961,903. Such ordered crystal structures generally contain 25 to 40 atomic % Al and alloying additions such as Zr, B, Mo, C, Cr, V, Nb, Si and Y.

An iron aluminide alloy having a disordered body centered crystal structure is disclosed in U.S. Pat. No. 5,238,645 wherein the alloy includes, in weight %, 8–9.5 Al,  $\leq 7$  Cr,  $\leq 4$  Mo,  $\leq 0.05$  C,  $\leq 0.5$  Zr and  $\leq 0.1$  Y, preferably 4.5–5.5 Cr, 1.8–2.2 Mo, 0.02–0.032 C and 0.15–0.25 Zr. Except for for three binary alloys having 8.46, 12.04 and 15.90 wt % Al, respectively, all of the specific alloy compositions disclosed in the '645 patent include a minimum of 5 wt % Cr. Further, the '645 patent states that the alloying elements improve strength, room-temperature ductility, high temperature oxidation resistance, aqueous corrosion resistance and resistance to pitting. The '645 patent does not relate to electrical resistance heating elements and does not address properties such as thermal fatigue resistance, electrical resistivity or high temperature sag resistance.

Iron-base alloys containing 3–18 wt % Al, 0.05–0.5 wt % Zr, 0.01–0.1 wt % B and optional Cr, Ti and Mo are disclosed in U.S. Pat. No. 3,026,197 and Canadian Pat. No. 648,140. The Zr and B are stated to provide grain refinement, the preferred Al content is 10–18 wt % and the alloys are disclosed as having oxidation resistance and workability. However, like the '645 patent, the '197 and Canadian patents do not relate to electrical resistance heating elements and do not address properties such as thermal fatigue resistance, electrical resistivity or high temperature sag resistance.

U.S. Pat. No. 3,676,109 discloses an iron-base alloy containing 3–10 wt % Al, 4–8 wt % Cr, about 0.5 wt % Cu, less than 0.05 wt % C, 0.5–2 wt % Ti and optional Mn and B. The '109 patent discloses that the Cu improves resistance to rust spotting, the Cr avoids embrittlement and the Ti provides precipitation hardening. The '109 patent states that the alloys are useful for chemical processing equipment. All of the specific examples disclosed in the '109 patent include 0.5 wt % Cu and at least 1 wt % Cr, with the preferred alloys having at least 9 wt % total Al and Cr, a minimum Cr or Al of at least 6 wt % and a difference between the Al and Cr contents of less than 6 wt %. However, like the '645 patent,

the '109 patent does not relate to electrical resistance heating elements and does not address properties such as thermal fatigue resistance, electrical resistivity or high temperature sag resistance.

5 Iron-base aluminum containing alloys for use as electrical resistance heating elements are disclosed in U.S. Pat. Nos. 1,550,508; 1,990,650; and 2,768,915 and in Canadian Patent No. 648,141. The alloys disclosed in the '508 patent include 20 wt % Al, 10 wt % Mn; 12–15 wt % Al, 6–8 wt % Mn; 10 or 12–16 wt % Al, 2–10 wt % Cr. All of the specific examples disclosed in the '508 patent include at least 6 wt % Cr and at least 10 wt % Al. The alloys disclosed in the '650 patent include 16–20 wt % Al, 5–10 wt % Cr,  $\leq 0.05$  wt % C,  $\leq 0.25$  wt % Si, 0.1–0.5 wt % Ti,  $\leq 1.5$  wt % Mo and 0.4–1.5 wt % Mn and the only specific example includes 17.5 wt % Al, 8.5 wt % Cr, 0.44 wt % Mn, 0.36 wt % Ti, 0.02 wt % C and 0.13 wt % Si. The alloys disclosed in the '915 patent include 10–18 wt % Al, 1–5 wt % Mo, Ti, Ta, V, Cb, Cr, Ni, B and W and the only specific example includes 16 wt % Al and 3 wt % Mo. The alloys disclosed in the Canadian patent include 6–11 wt % Al, 3–10 wt % Cr,  $\leq 4$  wt % Mn,  $\leq 1$  wt % Si,  $\leq 0.4$  wt % Ti,  $\leq 0.5$  wt % C, 0.2–0.5 wt % Zr and 0.05–0.1 wt % B and the only specific examples include at least 5 wt % Cr.

25 Resistance heaters of various materials are disclosed in U.S. Pat. No. 5,249,586 and in U.S. patent application Ser. Nos. 07/943,504, 08/118,665, 08/105,346 and 08/224,848.

U.S. Pat. No. 4,334,923 discloses a cold-rollable oxidation resistant iron-base alloy useful for catalytic converters containing  $\leq 0.05$  C, 0.1–2% Si, 2–8% Al, 0.02–1% Y,  $<0.009$  P,  $<0.006$  S and  $<0.009$  O.

U.S. Pat. No. 4,684,505 discloses a heat resistant iron-base alloy containing 10–22% Al, 2–12% Ti, 2–12% Mo, 0.1–1.2% Hf,  $\leq 1.5$  Si,  $\leq 0.3$  C,  $\leq 0.2$  B,  $\leq 1.0$  Ta,  $\leq 0.5$  W,  $\leq 0.5$  V,  $\leq 0.5$  Mn,  $\leq 0.3$  Co,  $\leq 0.3$  Nb, and  $\leq 0.2$  La. The '505 patent discloses a specific alloy having 16% Al, 0.5% Hf, 4% Mo, 3% Si, 4% Ti and 0.2% C.

40 Japanese Laid-open Patent Application No. 53–119721 discloses a wear resistant, high magnetic permeability alloy having good workability and containing 1.5–17% Al, 0.2–15% Cr and 0.01–8% total of optional additions of <4% Si, <8% Mo, <8% W, <8% Ti, <8% Ge, <8% Cu, <8% V, <8% Mn, <8% Nb, <8% Ta, <8% Ni, <8% Co, <3% Sn, <3% Sb, <3% Be, <3% Hf, <3% Zr, <0.5% Pb, and <3% rare earth metal. Except for a 16% Al, balance Fe alloy, all of the specific examples in Japan '721 include at least 1% Cr and except for a 5% Al, 3% Cr, balance Fe alloy, the remaining examples in Japan '721 include  $\geq 10$ % Al.

45 A 1990 publication in Advances in Powder Metallurgy, Vol. 2, by J. R. Knibloe et al., entitled "Microstructure And Mechanical Properties of P/M  $Fe_3Al$  Alloys", pp. 219–231, discloses a powder metallurgical process for preparing

50  $Fe_3Al$  containing 2 and 5% Cr by using an inert gas atomizer. This publication explains that  $Fe_3Al$  alloys have a  $DO_3$  structure at low temperatures and transform to a B2 structure above about 550° C. To make sheet, the powders were canned in mild steel, evacuated and hot extruded at 1000° C. to an area reduction ratio of 9:1. After removing from the steel can, the alloy extrusion was hot forged at 1000° C. to 0.340 inch thick, rolled at 800° C. to sheet approximately 0.10 inch thick and finish rolled at 650° C. to 0.030 inch. According to this publication, the atomized powders were generally spherical and provided dense extrusions and room temperature ductility approaching 20% was achieved by maximizing the amount of B2 structure.

A 1991 publication in Mat. Res. Soc. Symp. Proc., Vol. 213, by V. K. Sikka entitled "Powder Processing of  $Fe_3Al$ -Based Iron-Aluminide Alloys," pp. 901-906, discloses a process of preparing 2 and 5% Cr containing  $Fe_3Al$ -based iron-aluminide powders fabricated into sheet. This publication states that the powders were prepared by nitrogen-gas atomization and argon-gas atomization. The nitrogen-gas atomized powders had low levels of oxygen (130 ppm) and nitrogen (30 ppm). To make sheet, the powders were canned in mild steel and hot extruded at 1000° C. to an area reduction ratio of 9:1. The extruded nitrogen-gas atomized powder had a grain size of 30  $\mu m$ . The steel can was removed and the bars were forged 50% at 1000° C., rolled 50% at 850° C. and finish rolled 50% at 650° C. to 0.76 mm sheet.

A paper by V. K. Sikka et al., entitled "Powder Production, Processing, and Properties of  $Fe_3Al$ ", pp. 1-11, presented at the 1990 Powder Metallurgy Conference Exhibition in Pittsburgh, Pa., discloses a process of preparing  $Fe_3Al$  powder by melting constituent metals under a protective atmosphere, passing the metal through a metering nozzle and disintegrating the melt by impingement of the melt stream with nitrogen atomizing gas. The powder had low oxygen (130 ppm) and nitrogen (30 ppm) and was spherical. An extruded bar was produced by filling a 76 mm mild steel can with the powder, evacuating the can, heating 1½ hour at 1000° C. and extruding the can through a 25 mm die for a 9:1 reduction. The grain size of the extruded bar was 20  $\mu m$ . A sheet 0.76 mm thick was produced by removing the can, forging 50% at 1000° C., rolling 50% at 850° C. and finish rolling 50% at 650° C.

Oxide dispersion strengthened iron-base alloy powders are disclosed in U.S. Pat. Nos. 4,391,634 and 5,032,190. The '634 patent discloses Ti-free alloys containing 10-40% Cr, 1-10% Al and  $\leq 10\%$  oxide dispersoid. The '190 patent discloses a method of forming sheet from alloy MA 956 having 75% Fe, 20% Cr, 4.5% Al, 0.5% Ti and 0.5%  $Y_2O_3$ .

A publication by A. LeFort et al., entitled "Mechanical Behavior of  $FeAl_{40}$  Intermetallic Alloys" presented at the Proceedings of International Symposium on Intermetallic Compounds—Structure and Mechanical Properties (JIMIS-6), pp. 579-583, held in Sendai, Japan on Jun. 17-20, 1991, discloses various properties of  $FeAl$  alloys (25 wt % Al) with additions of boron, zirconium, chromium and cerium. The alloys were prepared by vacuum casting and extruding at 1100° C. or formed by compression at 1000° C. and 1100° C. This article explains that the excellent resistance of  $FeAl$  compounds in oxidizing and sulfidizing conditions is due to the high Al content and the stability of the B2 ordered structure.

A publication by D. Poccia et al., entitled "Production and Properties of CSM  $FeAl$  Intermetallic Alloys" presented at the Minerals, Metals and Materials Society Conference (1994 TMS Conference) on "Processing, Properties and Applications of Iron Aluminides", pp. 19-30, held in San Francisco, Calif. on Feb. 27-Mar. 3, 1994, discloses various properties of  $Fe_{40}Al$  intermetallic compounds processed by different techniques such as casting and extrusion, gas atomization of powder and extrusion and mechanical alloying of powder and extrusion and that mechanical alloying has been employed to reinforce the material with a fine oxide dispersion. The article states that  $FeAl$  alloys were prepared having a B2 ordered crystal structure, an Al content ranging from 23 to 25 wt % (about 40 at %) and alloying additions of Zr, Cr, Ce, C, B and  $Y_2O_3$ . The article states that the materials are candidates as structural materials in corrosive environments at high temperatures and will find use in

thermal engines, compressor stages of jet engines, coal gasification plants and the petrochemical industry.

A publication by J. H. Schneibel entitled "Selected Properties of Iron Aluminides", pp. 329-341, presented at the 1994 TMS Conference discloses properties of iron aluminides. This article reports properties such as melting temperatures, electrical resistivity, thermal conductivity, thermal expansion and mechanical properties of various  $FeAl$  compositions.

A publication by J. Baker entitled "Flow and Fracture of  $FeAl$ ", pp. 101-115, presented at the 1994 TMS Conference discloses an overview of the flow and fracture of the B2 compound  $FeAl$ . This article states that prior heat treatments strongly affect the mechanical properties of  $FeAl$  and that higher cooling rates after elevated temperature annealing provide higher room temperature yield strength and hardness but lower ductility due to excess vacancies. With respect to such vacancies, the article indicates that the presence of solute atoms tends to mitigate the retained vacancy effect and long term annealing can be used to remove excess vacancies.

A publication by D. J. Alexander entitled "Impact Behavior of  $FeAl$  Alloy FA-350", pp. 193-202, presented at the 1994 TMS Conference discloses impact and tensile properties of iron aluminide alloy FA-350. The FA-350 alloy includes, in atomic %, 35.8% Al, 0.2% Mo, 0.05% Zr and 0.13% C.

A publication by C. H. Kong entitled "The Effect of Ternary Additions on the Vacancy Hardening and Defect Structure of  $FeAl$ ", pp. 231-239, presented at the 1994 TMS Conference discloses the effect of ternary alloying additions on  $FeAl$  alloys. This article states that the B2 structured compound  $FeAl$  exhibits low room temperature ductility and unacceptably low high temperature strength above 500° C. The article states that room temperature brittleness is caused by retention of a high concentration of vacancies following high temperature heat treatments. The article discusses the effects of various ternary alloying additions such as Cu, Ni, Co, Mn, Cr, V and Ti as well as high temperature annealing and subsequent low temperature vacancy-relieving heat treatment.

A publication by D. J. Gaydosh et al., entitled "Microstructure and Tensile Properties of Fe-40 At.Pct. Al Alloys with C, Zr, Hf and B Additions" in the September 1989 Met. Trans A, Vol. 20A, pp. 1701-1714, discloses hot extrusion of gas-atomized powder wherein the powder either includes C, Zr and Hf as prealloyed additions or B is added to a previously prepared iron-aluminum powder.

A publication by C. G. McKamey et al., entitled "A review of recent developments in  $Fe_3Al$ -based Alloys" in the August 1991 J. of Mater. Res., Vol. 6, No. 8, pp. 1779-1805, discloses techniques for obtaining iron-aluminide powders by inert gas atomization and preparing ternary alloy powders based on  $Fe_3Al$  by mixing alloy powders to produce the desired alloy composition and consolidating by hot extrusion, i.e., preparation of  $Fe_3Al$ -based powders by nitrogen- or argon-gas atomization and consolidation to full density by extruding at 1000° C. to an area reduction of  $\leq 9:1$ .

Conventional powder metallurgical techniques of preparing iron-aluminides include melting iron and aluminum and inert gas atomizing the melt to form an iron-aluminide powder, canning the powder and working the canned material at elevated temperatures. It would be desirable if iron-aluminide could be prepared by a powder metallurgical technique wherein it is not necessary to can the powder and

wherein it is not necessary to prealloy the iron and aluminum in order to form iron-aluminide powder.

#### SUMMARY OF THE INVENTION

The invention provides a method of manufacturing an iron aluminide alloy by a powder metallurgical technique, comprising steps of preparing a mixture of aluminum powder and iron powder; shaping the mixture into an article; and sintering the article at a temperature sufficient to react the aluminum powder and the iron powder and form an iron aluminide. The aluminum powder can comprise an unalloyed aluminum powder and the iron powder can comprise an iron alloy, pure iron or mixture thereof. Binder can be added to the mixture prior to the shaping step. The method can include heating the article in a vacuum or inert atmosphere and removing volatile components from the article prior to the sintering step. For instance, the article can be heated to a temperature below 700° C. during the step of removing the volatile components. The aluminum and iron powders can have an average particle size of 10 to 60  $\mu\text{m}$ , preferably 40 to 60  $\mu\text{m}$ . The shaping can be carried out by cold rolling the powder mixture in direct contact with rollers of a rolling apparatus or by tape casting the powder mixture.

The iron-aluminide preferably has a ferritic structure which is austenite free. According to one embodiment of the invention, the iron aluminide can consist essentially of FeAl. Alternatively, the iron aluminide can be alloyed with other constituents and include, in weight %, 22.0–32.0% Al  $\leq$  2% Mo,  $\leq$  1% Zr,  $\leq$  2% Si,  $\leq$  30% Ni,  $<$  10% Cr,  $\leq$  0.1% C,  $\leq$  0.5% Y,  $\leq$  0.1% B,  $\leq$  1% Nb and  $\leq$  1% Ta. As examples, the iron aluminide can consist essentially of, in weight %, 22–32% Al, 0.3–0.5% Mo, 0.05–0.15% Zr, 0.01–0.05% C,  $\leq$  25%  $\text{Al}_2\text{O}_3$  particles,  $\leq$  1%  $\text{Y}_2\text{O}_3$  particles, balance Fe or 22–32% Al, 0.3–0.5% Mo, 0.05–0.3% Zr, 0.01–0.1% C,  $\leq$  1%  $\text{Y}_2\text{O}_3$ , balance Fe.

The shaping step preferably comprises cold rolling the powder mixture into a sheet. The method can further include forming the article (e.g., sheet) into an electrical resistance heating element subsequent to the sintering step, the electrical resistance heating element being capable of heating to 900° C. in less than 1 second when a voltage up to 10 volts and up to 6 amps is passed through the heating element. The sintering step can be carried out in first and second stages, the first stage comprising heating the article to a temperature at which up to one-half of the aluminum powder reacts with the iron powder to form  $\text{Fe}_3\text{Al}$ ,  $\text{Fe}_2\text{Al}_5$  or  $\text{FeAl}_3$ , and the second stage comprising heating the article to a temperature at which unreacted aluminum powder melts and reacts with the iron powder to form the FeAl. The article can be heated at a rate of no greater than 200° C./minute during the first stage and the article can be heated above 1200° C. during the second stage. The method can include working the article subsequent to the sintering step, such as by hot and/or cold rolling the article. The sintering step can produce a porosity of 25 to 40% in the article and the method can further comprise a step of working the article subsequent to the sintering step such that the porosity of the article is reduced to below 5% during the working step. The sheet can be reduced to a thickness of less than 0.010 inch during the rolling step.

#### BRIEF DESCRIPTION OF THE DRAWINGS

FIG. 1 shows the effect of changes in Al content on room-temperature properties of an aluminum containing iron-base alloy;

FIG. 2 shows the effect of changes in Al content on room temperature and high-temperature properties of an aluminum containing iron-base alloy;

FIG. 3 shows the effect of changes in Al content on high temperature stress to elongation of an aluminum containing iron-base alloy;

FIG. 4 shows the effect of changes in Al content on stress to rupture (creep) properties of an aluminum containing iron-base alloy;

FIG. 5 shows the effect of changes in Si content on room-temperature tensile properties of an Al and Si containing iron-base alloy;

FIG. 6 shows the effect of changes in Ti content on room-temperature properties of an Al and Ti containing iron-base alloy; and

FIG. 7 shows the effect of changes in Ti content on creep rupture properties of a Ti containing iron-base alloy.

FIGS. 8a–c show yield strength, ultimate tensile strength and total elongation for alloy numbers 23, 35, 46 and 48;

FIGS. 9a–c show yield strength, ultimate tensile strength and total elongation for commercial alloy Haynes 214 and alloys 46 and 48;

FIGS. 10a–b show ultimate tensile strength at tensile strain rates of  $3 \times 10^{-4}/\text{s}$  and  $3 \times 10^{-2}/\text{s}$ , respectively; and

FIGS. 10a–d show plastic elongation to rupture at strain rates of  $3 \times 10^{-4}/\text{s}$  and  $3 \times 10^{-2}/\text{s}$ , respectively, for alloys 57, 58, 60 and 61;

FIGS. 11a–b show yield strength and ultimate tensile strength, respectively, at 850° C. for alloys 46, 48 and 56, as a function of annealing temperatures;

FIGS. 12a–e show creep data for alloys 35, 46, 48 and 56, wherein FIG. 12a shows creep data for alloy 35 after annealing at 1050° C. for two hours in vacuum, FIG. 12b shows creep data for alloy 46 after annealing at 700° C. for one hour and air cooling, FIG. 12c shows creep data for alloy 48 after annealing at 1100° C. for one hour in vacuum and wherein the test is carried out at 1 ksi at 800° C., FIG. 12d shows the sample of FIG. 12c tested at 3 ksi and 800° C. and FIG. 12e shows alloy 56 after annealing at 1100° C. for one hour in vacuum and tested at 3 ksi and 800° C.;

FIGS. 13a–c show graphs of hardness (Rockwell C) values for alloys 48, 49, 51, 52, 53, 54 and 56 wherein FIG. 13a shows hardness versus annealing for 1 hour at temperatures of 750–1300° C. for alloy 48; FIG. 13b shows hardness versus annealing at 400° C. for times of 0–140 hours for alloys 49, 51 and 56; and FIG. 13c shows hardness versus annealing at 400° C. for times of 0–80 hours for alloys 52, 53 and 54;

FIGS. 14a–e show graphs of creep strain data versus time for alloys 48, 51 and 56, wherein FIG. 14a shows a comparison of creep strain at 800° C. for alloys 48 and 56, FIG. 14b shows creep strain at 800° C. for alloy 48, FIG. 14c shows creep strain at 800° C., 825° C. and 850° C. for alloy 48 after annealing at 1100° C. for one hour, FIG. 14d shows creep strain at 800° C., 825° C. and 850° C. for alloy 48 after annealing at 750° C. for one hour, and FIG. 14e shows creep strain at 850° C. for alloy 51 after annealing at 400° C. for 139 hours;

FIGS. 15a–b show graphs of creep strain data versus time for alloy 62 wherein FIG. 15a shows a comparison of creep strain at 850° C. and 875° C. for alloy 62 in the form of sheet and FIG. 15b shows creep strain at 800° C., 850° C. and 875° C. for alloy 62 in the form of bar; and

FIGS. 16a–b show graphs of electrical resistivity versus temperature for alloys 46 and 43 wherein FIG. 16a shows electrical resistivity of alloys 46 and 43 and FIG. 16b shows effects of a heating cycle on electrical resistivity of alloy 43.

#### DETAILED DESCRIPTION OF THE PREFERRED EMBODIMENTS

The invention provides a simple and economical powder metallurgical process for preparing iron-aluminide in desir-

able shapes such as sheet, bar, wire, or other desired shape of the material. In the process, a mixture of iron and aluminum powder is prepared, the mixture is shaped into an article and the article is sintered in order to react the iron and aluminum powders and form iron-aluminide. The shaping can be carried out at low temperature by cold rolling the powder without encasing the powder in a protective shell such as a metal can. The aluminum powder is preferably an unalloyed aluminum powder but the iron powder can be pure iron powder or an iron alloy powder. Moreover, additional alloying components can be mixed with the iron and aluminum powders when the mixture is formed.

Prior to shaping the article, a binder such as paraffin and/or a sintering aid is preferably added to the powder mixture. After the shaping step, it is desirable to remove volatile components in the article by heating the article to a suitable temperature to remove the volatile components. For instance, the article can be heated to a temperature in the range of 500 to 700° C., preferably 550 to 650° C. for a suitable time such as ½ to 1 hour in order to remove volatile components such as oxygen and carbon. The article can be heated in a vacuum or inert gas atmosphere such as an argon atmosphere and the heating is preferably at a rate of no more than 200° C./min. During this preliminary heating stage, some of the aluminum may react with the iron to form compounds such as  $Fe_3Al$  or  $Fe_2Al_5$  or  $FeAl_3$  and a minor amount of aluminum may react with the iron to form  $FeAl$ . However, during the sintering step iron and aluminum react to form the desired iron-aluminide such as  $FeAl$ .

The sintering step can be carried out at a temperature above 1200° C. in order to react the iron and aluminum to form the desired iron aluminide. The sintering is preferably carried out at a temperature of 1250 to 1300° C. for ½ to 2 hours in a vacuum or inert gas (e.g., Ar) atmosphere. During the sintering step, free aluminum melts and reacts with iron to form iron-aluminide.

The sintering step can produce substantial porosity in the sintered article, e.g., 25–40 vol % porosity. In order to reduce such porosity, the sintered article can be hot or cold rolled to reduce the thickness thereof and thereby increase the density and remove porosity in the article. If hot rolling is carried out, the hot rolling is preferably carried in an inert atmosphere or the article can be protected by a protective coating such as a ceramic or glass coating during the hot rolling step. If the article is subjected to cold rolling, it is not necessary to roll the article in a protective environment. Subsequent to the hot or cold rolling, the article can be annealed at a temperature of 1100–1200° C. in a vacuum or inert gas atmosphere for ½ to 2 hours. Then, the article can be further worked and/or annealed, as desired.

According to an example of the process according to the invention, a sheet of iron-aluminide containing 22–32 wt % Al (38–46 at % Al) is prepared as follows. First, a mixture of aluminum powder and iron powder along with optional alloying constituents is prepared, binder is added to the powder mixture and a compact is prepared for rolling or the mixture is fed directly to a rolling apparatus. The powder mixture is subjected to cold rolling to produce a sheet having a thickness of 0.022–0.030 inch. The rolled sheet is then heated at a rate of  $\leq 200$ ° C./min to 600° C. and held at this temperature in a vacuum or Ar atmosphere for ½ to 1 hour in order to drive off volatile components of the binders in the powder mixture. Subsequently, the temperature of the article is increased to 1250 to 1300° C. in the vacuum or argon atmosphere and the article is sintered for ½ to 2 hours. During the heating at 600° C., part of the aluminum reacts with iron to form  $Fe_3Al$ ,  $Fe_2Al_5$  and/or  $FeAl_3$  with only a

minor amount of  $FeAl$  being formed. During the sintering step at 1250 to 1300° C., remaining free aluminum melts and forms additional  $FeAl$  and the  $Fe_3Al$ ,  $Fe_2Al_5$  and  $FeAl_3$  compounds are converted to  $FeAl$ . The sintering results in a porosity of 25 to 40%. In order to remove the porosity, the sintered article is hot or cold rolled to a thickness of 0.008 inch. For instance, the sintered sheet can be cold rolled to about 0.012 inch, annealed at 1100 to 1200° C. for ½ to 2 hours in a vacuum or argon atmosphere, cold rolled to about 0.008 inch and again annealed at 1100 to 1200° C. for ½ to 2 hours in a vacuum or argon atmosphere. The finished sheet can then be processed further into electrical resistance heating elements.

The powder composition can be formed into a tape or sheet by a tape casting process. For instance, a layer of the powder composition can be deposited from a reservoir on a sheet of material (such as a cellulose acetate sheet) as the sheet is unwound from a roll. The thickness of the powder layer on the sheet can be controlled by one or more doctor blades which contact an upper surface of the powder layer as it travels on the sheet past the doctor blade(s). The powder composition preferably includes a binder which forms a tough but flexible film, volatilizes without leaving a residue in the powder, is not affected by ambient conditions during storage, is relatively inexpensive and/or is soluble in inexpensive yet volatile and non-flammable organic solvents. Selection of the binder may depend on tape thickness, casting surface and/or solvent desired.

For tape casting a thick layer of at least 0.01 inch thick, the binder can comprise 3 parts polyvinyl butyral (e.g., Butvar Type 13–76 sold by Monsanto, Co.), the solvent can comprise 35 parts toluene and the plasticizer can comprise 5.6 parts polyethylene glycol per 100 parts by weight powder. For tape casting a thin layer of less than 0.01 inch thick, the binder can comprise 15 parts vinyl chloride-acetate (e.g., VYNs, 90–10 vinyl chloride-vinyl acetate copolymer sold by Union Carbide Corp.), the solvent can comprise 85 parts MEK and the plasticizer can comprise 1 part butyl benzyl phthalate. If desired, the powder tape casting mixture can also include other ingredients such as deflocculants and/or wetting agents. Suitable binder, solvent, plasticizer, deflocculant and/or wetting agent compositions for tape casting in accordance with the invention will be apparent to the skilled artisan.

The method according to the invention can be used to prepare various iron aluminide alloys containing at least 4% by weight (wt %) of aluminum and having a  $Fe_3Al$  phase with a  $DO_3$  structure or an  $FeAl$  phase with a B2 structure. The alloys preferably are ferritic with an austenite-free microstructure and may contain one or more alloy elements selected from molybdenum, titanium, carbon, rare earth metal such as yttrium or cerium, boron, chromium, oxide such as  $Al_2O_3$  or  $Y_2O_3$ , and a carbide former (such as zirconium, niobium and/or tantalum) which is useable in conjunction with the carbon for forming carbide phases within the solid solution matrix for the purpose of controlling grain size and/or precipitation strengthening.

The aluminum concentration in the Fe-Al alloys can range from 14 to 32% by weight (nominal) and the Fe-Al alloys when wrought or powder metallurgically processed can be tailored to provide selected room temperature ductilities at a desirable level by annealing the alloys in a suitable atmosphere at a selected temperature greater than about 700° C. (e.g., 700–1100° C.) and then furnace cooling, air cooling or oil quenching the alloys while retaining yield and ultimate tensile strengths, resistance to oxidation and aqueous corrosion properties.

The concentration of the alloying constituents used in forming the Fe-Al alloys is expressed herein in nominal weight percent. However, the nominal weight of the aluminum in these alloys essentially corresponds to at least about 97% of the actual weight of the aluminum in the alloys. For example, a nominal 18.46 wt % may provide an actual 18.27 wt % of aluminum, which is about 99% of the nominal concentration.

The Fe-Al alloys can be processed or alloyed with one or more selected alloying elements for improving properties such as strength, room-temperature ductility, oxidation resistance, aqueous corrosion resistance, pitting resistance, thermal fatigue resistance, electrical resistivity, high temperature sag or creep resistance and resistance to weight gain. Effects of various alloying additions and processing are shown in the drawings, Tables 1-6 and following discussion.

The aluminum containing iron based alloys can be manufactured into electrical resistance heating elements. However, the alloy compositions disclosed herein can be used for other purposes such as in thermal spray applications wherein the alloys could be used as coatings having oxidation and corrosion resistance. Also, the alloys could be used as oxidation and corrosion resistant electrodes, furnace components, chemical reactors, sulfidization resistant materials, corrosion resistant materials for use in the chemical industry, pipe for conveying coal slurry or coal tar, substrate materials for catalytic converters, exhaust pipes for automotive engines, porous filters, etc.

According to one aspect of the invention, the geometry of the alloy can be varied to optimize heater resistance according to the formula:  $R = \rho (L/W \times T)$  wherein  $R$ =resistance of the heater,  $\rho$ =resistivity of the heater material,  $L$ =length of heater,  $W$ =width of heater and  $T$ =thickness of heater. The resistivity of the heater material can be varied by adjusting the aluminum content of the alloy, processing of the alloy or incorporating alloying additions in the alloy. For instance, the resistivity can be significantly increased by incorporating particles of alumina in the heater material. The alloy can optionally include other ceramic particles to enhance creep resistance and/or thermal conductivity. For instance, the heater material can include particles or fibers of electrically conductive material such as nitrides of transition metals (Zr, Ti, Hf), carbides of transition metals, borides of transition of metals and  $\text{MoSi}_2$  for purposes of providing good high temperature creep resistance up to 1200° C. and also excellent oxidation resistance. The heater material may also incorporate particles of electrically insulating material such as  $\text{Al}_2\text{O}_3$ ,  $\text{Y}_2\text{O}_3$ ,  $\text{Si}_3\text{N}_4$ ,  $\text{ZrO}_2$  for purposes of making the heater material creep resistant at high temperature and also enhancing thermal conductivity and/or reducing the thermal coefficient of expansion of the heater material. The electrically insulating/conductive particles/fibers can be added to a powder mixture of Fe, Al or iron aluminide or such particles/fibers can be formed by reaction synthesis of elemental powders which react exothermically during manufacture of the heater element.

The heater material can be made in various ways. For instance, the heater material can be made from a prealloyed powder, by mechanically alloying the alloy constituents or by reacting powders of iron and aluminum after a powder mixture thereof has been shaped into an article such as a sheet of cold rolled powder. The creep resistance of the material can be improved in various ways. For instance, a prealloyed powder can be mixed with  $\text{Y}_2\text{O}_3$  and mechanically alloyed so as to be sandwiched in the prealloyed powder. The mechanically alloyed powder can be processed by conventional powder metallurgical techniques such as by

canning and extruding, slip casting, centrifugal casting, hot pressing and hot isostatic pressing. Another technique is to use pure elemental powders of Fe, Al and optional alloying elements with or without ceramic particles such as  $\text{Y}_2\text{O}_3$  and cerium oxide and mechanically alloying such ingredients. In addition to the above, the above mentioned electrically insulating and/or electrically conductive particles can be incorporated in the powder mixture to tailor physical properties and high temperature creep resistance of the heater material.

The heater material can be made by conventional casting or powder metallurgy techniques. For instance, the heater material can be produced from a mixture of powder having different fractions but a preferred powder mixture comprises particles having a size smaller than minus 100 mesh. According to one aspect of the invention, the powder can be produced by gas atomization in which case the powder may have a spherical morphology. According to another aspect of the invention, the powder can be made by water atomization in which case the powder may have an irregular morphology. In addition, the powder produced by water atomization can include an aluminum oxide coating on the powder particles and such aluminum oxide can be broken up and incorporated in the heater material during thermomechanical processing of the powder to form shapes such as sheet, bar, etc. The alumina particles are effective in increasing resistivity of the iron aluminum alloy and while the alumina is effective in increasing strength and creep resistance, the ductility of the alloy is reduced.

When molybdenum is used as one of the alloying constituents it can be added in an effective range from more than incidental impurities up to about 5.0% with the effective amount being sufficient to promote solid solution hardening of the alloy and resistance to creep of the alloy when exposed to high temperatures. The concentration of the molybdenum can range from 0.25 to 4.25% and in one preferred embodiment is in the range of about 0.3 to 0.5%. Molybdenum additions greater than about 2.0% detract from the room-temperature ductility due to the relatively large extent of solid solution hardening caused by the presence of molybdenum in such concentrations.

Titanium can be added in an amount effective to improve creep strength of the alloy and can be present in amounts up to 3%. When present, the concentration of titanium is preferably in the range of  $\leq 2.0\%$ .

When carbon and the carbide former are used in the alloy, the carbon is present in an effective amount ranging from more than incidental impurities up to about 0.75% and the carbide former is present in an effective amount ranging from more than incidental impurities up to about 1.0% or more. The carbon concentration is preferably in the range of about 0.03% to about 0.3%. The effective amount of the carbon and the carbide former are each sufficient to together provide for the formation of sufficient carbides to control grain growth in the alloy during exposure thereof to increasing temperatures. The carbides may also provide some precipitation strengthening in the alloys. The concentration of the carbon and the carbide former in the alloy can be such that the carbide addition provides a stoichiometric or near stoichiometric ratio of carbon to carbide former so that essentially no excess carbon will remain in the finished alloy.

Zirconium can be incorporated in the alloy to improve high temperature oxidation resistance. If carbon is present in the alloy, an excess of a carbide former such as zirconium in the alloy is beneficial in as much as it will help form a

spallation-resistant oxide during high temperature thermal cycling in air. Zirconium is more effective than Hf since Zr forms oxide stringers perpendicular to the exposed surface of the alloy which pins the surface oxide whereas Hf forms oxide stringers which are parallel to the surface.

The carbide formers include such carbide-forming elements as zirconium, niobium, tantalum and hafnium and combinations thereof. The carbide former is preferably zirconium in a concentration sufficient for forming carbides with the carbon present within the alloy with this amount being in the range of about 0.02% to 0.6%. The concentrations for niobium, tantalum and hafnium when used as carbide formers essentially correspond to those of the zirconium.

In addition to the aforementioned alloy elements the use of an effective amount of a rare earth element such as about 0.05–0.25% cerium or yttrium in the alloy composition is beneficial since it has been found that such elements improve oxidation resistance of the alloy.

Improvement in properties can also be obtained by adding up to 30 wt % of oxide dispersoid particles such as  $Y_2O_3$ ,  $Al_2O_3$  or the like. The oxide dispersoid particles can be added to a melt or powder mixture of Fe, Al and other alloying elements. Alternatively, the oxide can be created in situ by water atomizing a melt of an aluminum-containing iron-based alloy whereby a coating of alumina or yttria on iron-aluminum powder is obtained. During processing of the powder, the oxides break up and are arranged as stringers in the final product. Incorporation of the oxide particles in the iron-aluminum alloy is effective in increasing the resistivity of the alloy. For instance, by incorporating about 0.5–0.6 wt % oxygen in the alloy, the resistivity can be raised from around 100  $\mu\Omega \cdot cm$  to about 160  $\mu\Omega \cdot cm$ .

In order to improve thermal conductivity and/or resistivity of the alloy, particles of electrically conductive and/or electrically insulating metal compounds can be incorporated in the alloy. Such metal compounds include oxides, nitrides, silicides, borides and carbides of elements selected from groups IVb, Vb and VIIb of the periodic table. The carbides can include carbides of Zr, Ta, Ti, Si, B, etc., the borides can include borides of Zr, Ta, Ti, Mo, etc., the silicides can include silicides of Mg, Ca, Ti, V, Cr, Mn, Zr, Nb, Mo, Ta, W, etc., the nitrides can include nitrides of Al, Si, Ti, Zr, etc., and the oxides can include oxides of Y, Al, Si, Ti, Zr, etc. In the case where the FeAl alloy is oxide dispersion strengthened, the oxides can be added to the powder mixture or formed in situ by adding pure metal such as Y to a molten metal bath whereby the Y can be oxidized in the molten bath, during atomization of the molten metal into powder and/or by subsequent treatment of the powder. For instance, the heater material can include particles of electrically conductive material such as nitrides of transition metals (Zr, Ti, Hf), carbides of transition metals, borides of transition of metals and  $MoSi_2$  for purposes of providing good high temperature creep resistance up to 1200° C. and also excellent oxidation resistance. The heater material may also incorporate particles of electrically insulating material such as  $Al_2O_3$ ,  $Y_2O_3$ ,  $Si_3N_4$ ,  $ZrO_2$  for purposes of making the heater material creep resistant at high temperature and also enhancing thermal conductivity and/or reducing the thermal coefficient of expansion of the heater material.

Additional elements which can be added to the alloys according to the invention include Si, Ni and B. For instance, small amounts of Si up to 2.0% can improve low and high temperature strength but room temperature and high temperature ductility of the alloy are adversely affected

with additions of Si above 0.25 wt %. The addition of up to 30 wt % Ni can improve strength of the alloy via second phase strengthening but Ni adds to the cost of the alloy and can reduce room and high temperature ductility thus leading to fabrication difficulties particularly at high temperatures. Small amounts of B can improve ductility of the alloy and B can be used in combination with Ti and/or Zr to provide titanium and/or zirconium boride precipitates for grain refinement. The effects to Al, Si and Ti are shown in FIGS. 1–7.

FIG. 1 shows the effect of changes in Al content on room temperature properties of an aluminum containing iron-base alloy. In particular, FIG. 1 shows tensile strength, yield strength, reduction in area, elongation and Rockwell A 15 hardness values for iron-base alloys containing up to 20 wt % Al.

FIG. 2 shows the effect of changes in Al content on high-temperature properties of an aluminum containing iron-base alloy. In particular, FIG. 2 shows tensile strength and proportional limit values at room temperature, 800° F., 1000° F., 1200° F. and 1350° F. for iron-base alloys containing up to 18 wt % Al.

FIG. 3 shows the effect of changes in Al content on high temperature stress to elongation of an aluminum containing iron-base alloy. In particular, FIG. 3 shows stress to  $\frac{1}{2}\%$  elongation and stress to 2% elongation in 1 hour for iron-base alloys containing up to 15–16 wt % Al.

FIG. 4 shows the effect of changes in Al content on creep properties of an aluminum containing iron-base alloy. In particular, FIG. 4 shows stress to rupture in 100 hour and 30 1000 hour for iron-base alloys containing up to 15–18 wt % Al.

FIG. 5 shows the effect of changes in Si content on room temperature tensile properties of an Al and Si containing iron-base alloy. In particular, FIG. 5 shows yield strength, tensile strength and elongation values for iron-base alloys containing 5.7 or 9 wt % Al and up to 2.5 wt % Si.

FIG. 6 shows the effect of changes in Ti content on room 40 temperature properties of an Al and Ti containing iron-base alloy. In particular, FIG. 6 shows tensile strength and elongation values for iron-base alloys containing up to 12 wt % Al and up to 3 wt % Ti.

FIG. 7 shows the effect of changes in Ti content on creep 45 rupture properties of a Ti containing iron-base alloy. In particular, FIG. 7 shows stress to rupture values for iron-base alloys containing up to 3 wt % Ti at temperatures of 700 to 1350° F.

FIGS. 8–16 shows graphs of properties of alloys in Tables 50 1a and 1b. FIGS. 8a–c show yield strength, ultimate tensile strength and total elongation for alloy numbers 23, 35, 46 and 48. FIGS. 9a–c show yield strength, ultimate tensile strength and total elongation for alloys 46 and 48 compared to commercial alloy Haynes 214. FIGS. 10a–b show ultimate tensile strength at tensile strain rates of  $3 \times 10^{-4}/s$  and  $3 \times 10^{-2}/s$ , respectively; and FIGS. 10a–c show plastic elongation to rupture at strain rates of  $3 \times 10^{-4}/s$  and  $3 \times 10^{-2}/s$ , respectively, for alloys 57, 58, 60 and 61. FIGS. 11a–b show yield strength and ultimate tensile strength, respectively, at 55 850° C. for alloys 46, 48 and 56, as a function of annealing temperatures. FIGS. 12a–e show creep data for alloys 35, 46, 48 and 56. FIG. 12a shows creep data for alloy 35 after annealing at 1050° C. for two hours in vacuum. FIG. 12b shows creep data for alloy 46 after annealing at 700° C. for one hour and air cooling. FIG. 12c shows creep data for alloy 48 after annealing at 1100° C. for one hour in vacuum and wherein the test is carried out at 1 ksi at 800° C. FIG. 60 65

12d shows the sample of FIG. 12c tested at 3 ksi and 800° C. and FIG. 12e shows alloy 56 after annealing at 1 100° C. for one hour in vacuum and tested at 3 ksi and 800° C.

FIGS. 13a-c show graphs of hardness (Rockwell C) values for alloys 48, 49, 51, 52, 53, 54 and 56 wherein FIG. 13a shows hardness versus annealing for 1 hour at temperatures of 750-1300° C. for alloy 48; FIG. 13b shows hardness versus annealing at 400° C. for times of 0-140 hours for alloys 49, 51 and 56; and FIG. 13c shows hardness versus annealing at 400° C. for times of 0-80 hours for alloys 52, 53 and 54.

FIGS. 14a-e show graphs of creep strain data versus time for alloys 48, 51 and 56, wherein FIG. 14a shows a comparison of creep strain at 800° C. for alloys 48 and 56, FIG. 14b shows creep strain at 800° C. for alloy 48, FIG. 14c shows creep strain at 800° C., 825° C. and 850° C. for alloy 48 after annealing at 1100° C. for one hour, FIG. 14d shows creep strain at 800° C., 825° C. and 850° C. for alloy 48 after annealing at 750° C. for one hour, and FIG. 14e shows creep strain at 850° C. for alloy 51 after annealing at 400° C. for 139 hours. FIGS. 15a-b show graphs of creep strain data versus time for alloy 62 wherein FIG. 15a shows a comparison of creep strain at 850° C. and 875° C. for alloy 62 in the form of sheet and FIG. 15b shows creep strain at 800° C., 850° C. and 875° C. for alloy 62 in the form of bar.

FIGS. 16a-b show graphs of electrical resistivity versus temperature for alloys 46 and 43 wherein FIG. 16a shows electrical resistivity of alloys 46 and 43 and FIG. 16b shows effects of a heating cycle on electrical resistivity of alloy 43.

The Fe-Al alloys can be formed by powder metallurgical techniques or by the arc melting, air induction melting, or vacuum induction melting of powdered and/or solid pieces of the selected alloy constituents at a temperature of about 1600° C. in a suitable crucible formed of ZrO<sub>2</sub> or the like. The molten alloy is preferably cast into a mold of graphite or the like in the configuration of a desired product or for forming a heat of the alloy used for the formation of an alloy article by working the alloy.

The melt of the alloy to be worked is cut, if needed, into an appropriate size and then reduced in thickness by forging at a temperature in the range of about 900 to 1100° C., hot rolling at a temperature in the range of about 750 to 1100° C., warm rolling at a temperature in the range of about 600 to 700° C., and/or cold rolling at room temperature. Each pass through the cold rolls can provide a 20 to 30% reduction in thickness and is followed by heat treating the alloy in air, inert gas or vacuum at a temperature in the range of about 700 to 1,050° C., preferably about 800° C. for one hour.

Wrought alloy specimens set forth in the following tables were prepared by arc melting the alloy constituents to form heats of the various alloys. These heats were cut into 0.5 inch thick pieces which were forged at 1000° C. to reduce the thickness of the alloy specimens to 0.25 inch (50% reduction), then hot rolled at 800° C. to further reduce the thickness of the alloy specimens to 0.1 inch (60% reduction), and then warm rolled at 650° C. to provide a final thickness of 0.030 inch (70% reduction) for the alloy specimens described and tested herein. For tensile tests, the specimens were punched from 0.030 inch sheet with a 1/2 inch gauge length of the specimen aligned with the rolling direction of the sheet.

Specimens prepared by powder metallurgical techniques are also set forth in the following tables. In general, powders were obtained by gas atomization or water atomization techniques. Depending on which technique is used, powder

morphology ranging from spherical (gas atomized powder) to irregular (water atomized powder) can be obtained. The water atomized powder includes an aluminum oxide coating which is broken up into stringers of oxide particles during thermomechanical processing of the powder into useful shapes such as sheet, strip, bar, etc. The oxide particles modify the electrical resistivity of the alloy by acting as discrete insulators in a conductive Fe-Al matrix.

10

S In order to compare compositions of alloys, alloy compositions are set forth in Tables 1 a-b. Table 2 sets forth strength and ductility properties at low and high temperatures for selected alloy compositions in Tables 1 a-b.

Sag resistance data for various alloys is set forth in Table 3. The sag tests were carried out using strips of the various alloys supported at one end or supported at both ends. The amount of sag was measured after heating the strips in an air atmosphere at 900° C. for the times indicated.

25

Creep data for various alloys is set forth in Table 4. The creep tests were carried out using a tensile test to determine stress at which samples ruptured at test temperature in 10 h, 100 h and 1000 h.

Electrical resistivity at room temperature and crystal structure for selected alloys are set forth in Table 5. As shown therein, the electrical resistivity is affected by composition and processing of the alloy.

40

Table 6 sets forth hardness data of oxide dispersion strengthened alloys in accordance with the invention. In particular, Table 6 shows the hardness (Rockwell C) of alloys 62, 63 and 64. As shown therein, even with up to 20% Al<sub>2</sub>O<sub>3</sub> (alloy 64), the hardness of the material can be maintained below Rc45. In order to provide workability, however, it is preferred that the hardness of the material be maintained below about Rc35. Thus, when it is desired to utilize oxide dispersion strengthened material as the resistance heater material, workability of the material can be improved by carrying out a suitable heat treatment to lower the hardness of the material.

55

Table 7 shows heats of formation of selected intermetallics which can be formed by reaction synthesis. While only aluminides and silicides are shown in Table 7, reaction synthesis can also be used to form carbides, nitrides, oxides and borides. For instance, a matrix of iron aluminide and/or electrically insulating or electrically conductive covalent ceramics in the form of particles or fibers can be formed by mixing elemental powders which react exothermically during heating of such powders. Thus, such reaction synthesis can be carried out while extruding or sintering powder used to form the heater element according to the invention.

60

65

TABLE 1

| Alloy |       | Composition In Weight % |      |     |     |     |      |      |      |      |      |     |    |    |    |   |
|-------|-------|-------------------------|------|-----|-----|-----|------|------|------|------|------|-----|----|----|----|---|
| No.   | Fe    | Al                      | Si   | Ti  | Mo  | Zr  | C    | Ni   | Y    | B    | Nb   | Ta  | Cr | Ce | Cu | O |
| 1     | 91.5  | 8.5                     |      |     |     |     |      |      |      |      |      |     |    |    |    |   |
| 2     | 91.5  | 6.5                     | 2.0  |     |     |     |      |      |      |      |      |     |    |    |    |   |
| 3     | 90.5  | 8.5                     |      |     | 1.0 |     |      |      |      |      |      |     |    |    |    |   |
| 4     | 90.27 | 8.5                     |      |     | 1.0 | 0.2 | 0.03 |      |      |      |      |     |    |    |    |   |
| 5     | 90.17 | 8.5                     | 0.1  | 1.0 |     | 0.2 | 0.03 |      |      |      |      |     |    |    |    |   |
| 6     | 89.27 | 8.5                     |      |     | 1.0 | 1.0 | 0.2  | 0.03 |      |      |      |     |    |    |    |   |
| 7     | 89.17 | 8.5                     | 0.1  | 1.0 | 1.0 | 0.2 | 0.03 |      |      |      |      |     |    |    |    |   |
| 8     | 93    | 6.5                     | 0.5  |     |     |     |      |      |      |      |      |     |    |    |    |   |
| 9     | 94.5  | 5.0                     | 0.5  |     |     |     |      |      |      |      |      |     |    |    |    |   |
| 10    | 92.5  | 6.5                     | 1.0  |     |     |     |      |      |      |      |      |     |    |    |    |   |
| 11    | 75.0  | 5.0                     |      |     |     |     | 20.0 |      |      |      |      |     |    |    |    |   |
| 12    | 71.5  | 8.5                     |      |     |     |     | 20.0 |      |      |      |      |     |    |    |    |   |
| 13    | 72.25 | 5.0                     | 0.5  | 1.0 | 1.0 | 0.2 | 0.03 | 20.0 | 0.02 |      |      |     |    |    |    |   |
| 14    | 76.19 | 6.0                     | 0.5  | 1.0 | 1.0 | 0.2 | 0.03 | 15.0 | 0.08 |      |      |     |    |    |    |   |
| 15    | 81.19 | 6.0                     | 0.5  | 1.0 | 1.0 | 0.2 | 0.03 | 10.0 | 0.08 |      |      |     |    |    |    |   |
| 16    | 86.23 | 8.5                     |      | 1.0 | 4.0 | 0.2 | 0.03 |      | 0.04 |      |      |     |    |    |    |   |
| 17    | 88.77 | 8.5                     |      | 1.0 | 1.0 | 0.6 | 0.09 |      | 0.04 |      |      |     |    |    |    |   |
| 18    | 85.77 | 8.5                     |      | 1.0 | 1.0 | 0.6 | 0.09 | 3.0  | 0.04 |      |      |     |    |    |    |   |
| 19    | 83.77 | 8.5                     |      | 1.0 | 1.0 | 0.6 | 0.09 | 5.0  | 0.04 |      |      |     |    |    |    |   |
| 20    | 88.13 | 8.5                     |      | 1.0 | 1.0 | 0.2 | 0.03 |      | 0.04 | 0.5  | 0.5  |     |    |    |    |   |
| 21    | 61.48 | 8.5                     |      |     |     |     | 30.0 |      | 0.02 |      |      |     |    |    |    |   |
| 22    | 88.90 | 8.5                     | 0.1  | 1.0 | 1.0 | 0.2 | 0.3  |      |      |      |      |     |    |    |    |   |
| 23    | 87.60 | 8.5                     | 0.1  | 2.0 | 1.0 | 0.2 | 0.6  |      |      |      |      |     |    |    |    |   |
| 24    | bal   | 8.19                    |      |     |     |     |      |      |      |      | 2.13 |     |    |    |    |   |
| 25    | bal   | 8.30                    |      |     |     |     |      |      |      |      | 4.60 |     |    |    |    |   |
| 26    | bal   | 8.28                    |      |     |     |     |      |      |      |      | 6.93 |     |    |    |    |   |
| 27    | bal   | 8.22                    |      |     |     |     |      |      |      |      | 9.57 |     |    |    |    |   |
| 28    | bal   | 7.64                    |      |     |     |     |      |      |      |      | 7.46 |     |    |    |    |   |
| 29    | bal   | 7.47                    | 0.32 |     |     |     |      |      |      |      | 7.53 |     |    |    |    |   |
| 30    | 84.75 | 8.0                     |      |     | 6.0 | 0.8 | 0.1  |      |      | 0.25 |      | 0.1 |    |    |    |   |
| 31    | 85.10 | 8.0                     |      |     | 6.0 | 0.8 | 0.1  |      |      |      |      |     |    |    |    |   |
| 32    | 86.00 | 8.0                     |      |     |     |     | 6.0  |      |      |      |      |     |    |    |    |   |

| Alloy |         | Composition In Weight % |     |      |       |       |        |        |      |                             |      |   |         |  |
|-------|---------|-------------------------|-----|------|-------|-------|--------|--------|------|-----------------------------|------|---|---------|--|
| No.   | Fe      | Al                      | Ti  | Mo   | Zr    | C     | Y      | B      | Cr   | Ce                          | Cu   | O | Ceramic |  |
| 33    | 78.19   | 21.23                   | —   | 0.42 | 0.10  | —     | —      | 0.060  | —    |                             |      |   |         |  |
| 34    | 79.92   | 19.50                   | —   | 0.42 | 0.10  | —     | —      | 0.060  | —    |                             |      |   |         |  |
| 35    | 81.42   | 18.00                   | —   | 0.42 | 0.10  | —     | —      | 0.060  | —    |                             |      |   |         |  |
| 36    | 82.31   | 15.00                   | 1.0 | 1.0  | 0.60  | 0.09  | —      | —      | —    |                             |      |   |         |  |
| 37    | 78.25   | 21.20                   | —   | 0.42 | 0.10  | 0.03  | —      | 0.005  | —    |                             |      |   |         |  |
| 38    | 78.24   | 21.20                   | —   | 0.42 | 0.10  | 0.03  | —      | 0.010  | —    |                             |      |   |         |  |
| 39    | 84.18   | 15.82                   | —   | —    | —     | —     | —      | —      | —    |                             |      |   |         |  |
| 40    | 81.98   | 15.84                   | —   | —    | —     | —     | —      | —      | 2.18 |                             |      |   |         |  |
| 41    | 78.66   | 15.88                   | —   | —    | —     | —     | —      | —      | —    | 5.46                        |      |   |         |  |
| 42    | 74.20   | 15.93                   | —   | —    | —     | —     | —      | —      | —    | 9.87                        |      |   |         |  |
| 43    | 78.35   | 21.10                   | —   | 0.42 | 0.10  | 0.03  | —      | —      | —    |                             |      |   |         |  |
| 44    | 78.35   | 21.10                   | —   | 0.42 | 0.10  | 0.03  | —      | 0.0025 | —    |                             |      |   |         |  |
| 45    | 78.58   | 21.26                   | —   | —    | 0.10  | —     | —      | 0.060  | —    |                             |      |   |         |  |
| 46    | 82.37   | 17.12                   | —   | —    | —     | —     | 0.010  | —      | —    | 0.50                        |      |   |         |  |
| 47    | 81.19   | 16.25                   | —   | —    | —     | —     | 0.015  | 2.22   | —    | —                           | 0.33 |   |         |  |
| 48    | 76.450  | 23.0                    | —   | 0.42 | 0.10  | 0.03  | —      | —      | —    | —                           | —    | — |         |  |
| 49    | 76.445  | 23.0                    | —   | 0.42 | 0.10  | 0.03  | —      | 0.005  | —    | —                           | —    | — |         |  |
| 50    | 76.243  | 23.0                    | —   | 0.42 | 0.10  | 0.03  | 0.2    | 0.005  | —    | —                           | —    | — |         |  |
| 51    | 75.445  | 23.0                    | 1.0 | 0.42 | 0.10  | 0.03  | —      | 0.005  | —    | —                           | —    | — |         |  |
| 52    | 74.8755 | 25.0                    | —   | —    | 0.10  | 0.023 | —      | 0.0015 | —    | —                           | —    | — |         |  |
| 53    | 72.8755 | 25.0                    | —   | —    | 0.10  | 0.023 | —      | 0.0015 | —    | 2.0                         | —    |   |         |  |
| 54    | 73.8755 | 25.0                    | 1.0 | —    | 0.10  | 0.023 | —      | 0.0015 | —    | —                           | —    | — |         |  |
| 55    | 73.445  | 26.0                    | —   | 0.42 | 0.10  | 0.03  | —      | 0.0015 | —    | —                           | —    | — |         |  |
| 56    | 69.315  | 30.0                    | —   | 0.42 | 0.20  | 0.06  | —      | 0.005  |      |                             |      |   |         |  |
| 57    | bal.    | 25                      |     |      | 0.10  | 0.023 | —      | 0.0015 | —    | —                           |      |   |         |  |
| 58    | bal.    | 24                      |     | —    | 0.010 | —     | 0.0030 | 2      | —    |                             |      |   |         |  |
| 59    | bal.    | 24                      |     | —    | 0.015 | —     | 0.0030 | <0.1   | —    |                             |      |   |         |  |
| 60    | bal.    | 24                      |     | —    | 0.015 | —     | 0.0025 | 5      | 0.5  |                             |      |   |         |  |
| 61    | bal.    | 25                      |     | —    |       | —     | 0.0030 | 2      | 0.1  |                             |      |   |         |  |
| 62    | bal.    | 23                      |     | 0.42 | 0.10  | 0.03  |        |        |      | 0.20 $\text{Y}_2\text{O}_3$ |      |   |         |  |
| 63    | bal.    | 23                      |     | 0.42 | 0.10  | 0.03  |        |        |      | 10 $\text{Al}_2\text{O}_3$  |      |   |         |  |
| 64    | bal.    | 23                      |     | 0.42 | 0.10  | 0.03  |        |        |      | 20 $\text{Al}_2\text{O}_3$  |      |   |         |  |
| 65    | bal.    | 24                      |     | 0.42 | 0.10  | 0.03  |        |        |      | 2 $\text{Al}_2\text{O}_3$   |      |   |         |  |
| 66    | bal.    | 24                      |     | 0.42 | 0.10  | 0.03  |        |        |      | 4 $\text{Al}_2\text{O}_3$   |      |   |         |  |
| 67    | bal.    | 24                      |     | 0.42 | 0.10  | 0.03  |        |        |      | 2 $\text{TiC}$              |      |   |         |  |
| 68    | bal.    | 24                      |     | 0.42 | 0.10  | 0.03  |        |        |      | 2 $\text{ZrO}_2$            |      |   |         |  |



TABLE 3

| Ends of<br>Supported | Sample           | Thickness<br>(mil) | Length of<br>Heating (h) | Amount of Sag (inch) |             |             |             |             |
|----------------------|------------------|--------------------|--------------------------|----------------------|-------------|-------------|-------------|-------------|
|                      |                  |                    |                          | Alloy<br>17          | Alloy<br>20 | Alloy<br>22 | Alloy<br>45 | Alloy<br>47 |
|                      | One <sup>a</sup> | 30                 | 16                       | 1/8                  | —           | —           | 1/8         | —           |
|                      | One <sup>b</sup> | 30                 | 21                       | —                    | 3/8         | 1/8         | 1/4         | —           |
|                      | Both             | 30                 | 185                      | —                    | 0           | 0           | 1/16        | 0           |
|                      | Both             | 10                 | 68                       | —                    | —           | 1/8         | 0           | 0           |

## Additional Conditions

<sup>a</sup>= wire weight hung on free end to make samples have same weight<sup>b</sup>= foils of same length and width placed on samples to make samples have same weight

TABLE 4

| Sample | Test<br>Temperature |      | Creep Rupture Strength (ksi) |       |        |
|--------|---------------------|------|------------------------------|-------|--------|
|        | ° F.                | ° C. | 10 h                         | 100 h | 1000 h |
| 1      | 1400                | 760  | 2.90                         | 2.05  | 1.40   |
|        | 1500                | 816  | 1.95                         | 1.35  | 0.95   |
|        | 1600                | 871  | 1.20                         | 0.90  | —      |
|        | 1700                | 925  | 0.90                         | —     | —      |
| 4      | 1400                | 760  | 3.50                         | 2.50  | 1.80   |
|        | 1500                | 816  | 2.40                         | 1.80  | 1.20   |
|        | 1600                | 871  | 1.65                         | 1.15  | —      |
|        | 1700                | 925  | 1.15                         | —     | —      |
| 5      | 1400                | 760  | 3.60                         | 2.50  | 1.85   |
|        | 1500                | 816  | 2.40                         | 1.80  | 1.20   |
|        | 1600                | 871  | 1.65                         | 1.15  | —      |
|        | 1700                | 925  | 1.15                         | —     | —      |
| 6      | 1400                | 760  | 3.50                         | 2.60  | 1.95   |
|        | 1500                | 816  | 2.50                         | 1.90  | 1.40   |
|        | 1600                | 871  | 1.80                         | 1.30  | —      |
|        | 1700                | 925  | 1.30                         | —     | —      |
| 7      | 1400                | 760  | 3.90                         | 2.90  | 2.15   |
|        | 1500                | 816  | 2.80                         | 2.00  | 1.65   |
|        | 1600                | 871  | 2.00                         | 1.50  | —      |
|        | 1700                | 925  | 1.50                         | —     | —      |
| 17     | 1400                | 760  | 3.95                         | 3.0   | 2.3    |
|        | 1500                | 816  | 2.95                         | 2.20  | 1.75   |
|        | 1600                | 871  | 2.05                         | 1.65  | 1.25   |
|        | 1700                | 925  | 1.65                         | 1.20  | —      |
| 20     | 1400                | 760  | 4.90                         | 3.25  | 2.05   |
|        | 1500                | 816  | 3.20                         | 2.20  | 1.65   |
|        | 1600                | 871  | 2.10                         | 1.55  | 1.0    |
|        | 1700                | 925  | 1.56                         | 0.95  | —      |
| 22     | 1400                | 760  | 4.70                         | 3.60  | 2.65   |
|        | 1500                | 816  | 3.55                         | 2.60  | 1.35   |
|        | 1600                | 871  | 2.50                         | 1.80  | 1.25   |
|        | 1700                | 925  | 1.80                         | 1.20  | 1.0    |

TABLE 5

| Alloy | Condition | Electrical Resistivity<br>Room-temp $\mu\Omega \cdot \text{cm.}$ | Crystal<br>Structure |
|-------|-----------|------------------------------------------------------------------|----------------------|
| 35    |           | 184                                                              | DO <sub>3</sub>      |
| 46    | A         | 167                                                              | DO <sub>3</sub>      |
| 46    | A + D     | 169                                                              | DO <sub>3</sub>      |
| 46    | A + E     | 181                                                              | B <sub>2</sub>       |
| 39    |           | 149                                                              | DO <sub>3</sub>      |
| 40    |           | 164                                                              | DO <sub>3</sub>      |
| 40    | B         | 178                                                              | DO <sub>3</sub>      |
| 41    | C         | 190                                                              | DO <sub>3</sub>      |
| 43    | C         | 185                                                              | B <sub>2</sub>       |
| 44    | C         | 178                                                              | B <sub>2</sub>       |
| 45    | C         | 184                                                              | B <sub>2</sub>       |
| 62    | F         | 197                                                              |                      |
| 63    | F         | 251                                                              |                      |
| 64    | F         | 337                                                              |                      |
| 65    | F         | 170                                                              |                      |

TABLE 5-continued

| 5 | Alloy | Condition | Electrical Resistivity<br>Room-temp $\mu\Omega \cdot \text{cm.}$ | Crystal<br>Structure |
|---|-------|-----------|------------------------------------------------------------------|----------------------|
|   | 66    | F         | 180                                                              |                      |
|   | 67    | F         | 158                                                              |                      |
|   | 68    | F         | 155                                                              |                      |

## Condition of Samples

A = water atomized powder

B = gas atomized powder

C = cast and processed

D = 1/2 hr. anneal at 700° C. + oil quench

E = 1/2 hr. anneal at 750° C. + oil quench

F = reaction synthesis to form covalent ceramic addition

TABLE 6

| 20                                                                                                                                                                                                                 | HARDNESS DATA |          |          |          |
|--------------------------------------------------------------------------------------------------------------------------------------------------------------------------------------------------------------------|---------------|----------|----------|----------|
| 25                                                                                                                                                                                                                 | CONDITION     | Alloy 62 | Alloy 63 | Alloy 64 |
| As extruded                                                                                                                                                                                                        |               | 39       | 37       | 44       |
| Annealed 750° C. for 1 h followed by slow cooling                                                                                                                                                                  |               | 35       | 34       | 44       |
| Alloy 62: Extruded in carbon steel at 1100° C. to a reduction ratio of 16:1 (2-to 1/2-in. die);<br>Alloy 63 and Alloy 64: Extruded in stainless steel at 1250° C. to a reduction ratio of 16:1 (2 to 1/2-in. die). |               |          |          |          |

TABLE 7

| 30 | Intermetallic                   | $\Delta H^\circ 298$ (K cal/mole) |
|----|---------------------------------|-----------------------------------|
| 35 | NiAl <sub>3</sub>               | -36.0                             |
|    | NiAl                            | -28.3                             |
|    | Ni <sub>2</sub> Al <sub>3</sub> | -67.5                             |
|    | Ni <sub>3</sub> Al              | -36.6                             |
| 40 | —                               | —                                 |
|    | FeAl <sub>3</sub>               | -18.9                             |
|    | FeAl                            | -12.0                             |
|    | —                               | —                                 |
|    | CoAl                            | -26.4                             |
|    | CoAl <sub>4</sub>               | -38.5                             |
|    | Co <sub>2</sub> Al <sub>5</sub> | -70.0                             |
| 45 | —                               | —                                 |
|    | Ti <sub>3</sub> Al              | -23.5                             |
|    | TiAl                            | -17.4                             |
|    | TiAl <sub>3</sub>               | -34.0                             |
|    | Ti <sub>2</sub> Al <sub>3</sub> | -27.9                             |
|    | —                               | —                                 |
|    | NbAl <sub>3</sub>               | -28.4                             |
|    | —                               | —                                 |
| 50 | TaAl                            | -19.2                             |
|    | TaAl <sub>3</sub>               | -26.1                             |
|    | Ni <sub>2</sub> Si              | -34.1                             |
|    | Ni <sub>3</sub> Si              | -55.5                             |
|    | NiSi                            | -21.4                             |
|    | NiSi <sub>2</sub>               | -22.5                             |
| 55 | —                               | —                                 |
|    | Mo <sub>3</sub> Si              | -27.8                             |
|    | Mo <sub>5</sub> Si <sub>3</sub> | -74.1                             |
|    | MoSi <sub>2</sub>               | -31.5                             |
| 60 | —                               | —                                 |
|    | Cr <sub>3</sub> Si              | -22.0                             |
|    | Cr <sub>5</sub> Si <sub>3</sub> | -50.5                             |
|    | CrSi                            | -12.7                             |
|    | CrSi <sub>2</sub>               | -19.1                             |
| 65 | —                               | —                                 |
|    | Co <sub>2</sub> Si              | -28.0                             |
|    | CoSi                            | -22.7                             |
|    | CoSi <sub>2</sub>               | -23.6                             |
|    | FeSi                            | -18.3                             |

TABLE 7-continued

| Intermetallic                   | $\Delta H^\circ$ 298 (K cal/mole) |
|---------------------------------|-----------------------------------|
| —                               | —                                 |
| NbSi <sub>2</sub>               | -33.0                             |
| Ta <sub>2</sub> Si              | -30.0                             |
| Ta <sub>5</sub> Si <sub>3</sub> | -80.0                             |
| TaSi                            | -28.5                             |
| —                               | —                                 |
| Ti <sub>2</sub> Si <sub>3</sub> | -138.5                            |
| TiSi                            | -31.0                             |
| TiSi <sub>2</sub>               | -32.1                             |
| —                               | —                                 |
| WSi <sub>2</sub>                | -22.2                             |
| W <sub>5</sub> Si <sub>3</sub>  | -32.3                             |
| —                               | —                                 |
| Zr <sub>2</sub> Si              | -81.0                             |
| Zr <sub>5</sub> Si <sub>3</sub> | -146.7                            |
| ZrSi                            | -35.3                             |
| —                               | —                                 |
| —                               | —                                 |
| —                               | —                                 |
| —                               | —                                 |
| —                               | —                                 |
| —                               | —                                 |

The foregoing has described the principles, preferred embodiments and modes of operation of the present invention. However, the invention should not be construed as being limited to the particular embodiments discussed. Thus, the above-described embodiments should be regarded as illustrative rather than restrictive, and it should be appreciated that variations may be made in those embodiments by workers skilled in the art without departing from the scope of the present invention as defined by the following claims.

What is claimed is:

1. A method of manufacturing an iron aluminide alloy by a powder metallurgical technique, comprising steps of: preparing a powder mixture of aluminum powder and iron powder; shaping the powder mixture into an article; sintering the article at a temperature sufficient to melt the aluminum powder and react the melted aluminum powder with the iron powder and form an iron aluminide. 35
  2. The method of claim 1, wherein the aluminum powder comprises an unalloyed aluminum powder and the iron powder comprises an iron alloy, pure iron or mixture thereof. 40
  3. The method of claim 1, wherein binder and one or more optional alloying constituents are added to the powder mixture prior to the shaping step. 45
  4. The method of claim 1, wherein the shaping is carried out by cold rolling the powder mixture into a sheet. 50
  5. The method of claim 1, further comprising heating the article in a vacuum or inert atmosphere and removing volatile components from the article prior to the sintering step. 55
  6. The method of claim 1, wherein the article is heated to a temperature below 700° C. during the step of removing the volatile components. 60
  7. The method of claim 1, wherein the iron aluminide consists essentially of FeAl. 65
  8. The method of claim 1, wherein the iron aluminide comprises, in weight %, 22.0-32.0% Al and ≤1% Cr.
  9. The method of claim 1, wherein the iron aluminide has a ferritic microstructure which is austenite-free.
  10. The method of claim 1, wherein the shaping step is carried out by cold rolling the powder mixture.
  11. The method of claim 1, further comprising forming the article into an electrical resistance heating element subsequent to the sintering step, the electrical resistance heating
- 5 element being capable of heating to 900° C. in less than 1 second when a voltage up to 10 volts and up to 6 amps is passed through the heating element.
12. A method of manufacturing an iron aluminide alloy by a powder metallurgical technique, comprising the steps of: preparing a powder mixture of aluminum powder and iron powder; shaping the powder mixture into an article; sintering the article at a temperature sufficient to react the aluminum powder and the iron powder and form an iron aluminide; and the sintering step is carried out in first and second stages, the first stage comprising heating the article to a temperature at which up to one-half of the aluminum powder reacts with the iron powder to form Fe<sub>3</sub>Al, Fe<sub>2</sub>Al<sub>5</sub>, FeAl<sub>3</sub> or mixtures thereof, and the second stage comprising heating the article to a temperature at which unreacted aluminum powder melts and reacts with the iron powder to form the iron aluminide. 10
  13. The method of claim 12, wherein the article is heated at a rate of no greater than 200° C./minute during the first stage. 15
  14. The method of claim 12, wherein the article is heated above 1200° C. during the second stage.
  15. The method of claim 1, further comprising working the article subsequent to the sintering step. 20
  16. The method of claim 15, wherein the working comprises hot and/or cold rolling the article. 25
  17. The method of claim 1, wherein the sintering step produces a porosity of 25 to 40% in the article, the method further comprising a step of working the article subsequent to the sintering step, the porosity of the article being reduced to below 5% during the working step. 30
  18. A method of manufacturing an iron aluminide alloy by a powder metallurgical technique, comprising the steps of: preparing a powder mixture of aluminum powder and iron powder; shaping the powder mixture into an article; sintering the article at a temperature sufficient to react the aluminum powder and the iron powder and form an iron aluminide; and the article comprises a sheet, the sheet being subjected to a rolling step followed by a heat treating step subsequent to the sintering step, the heat treating step being carried out at a temperature of 1100 to 1200° C. in a vacuum or inert atmosphere. 35
  19. The method of claim 18, wherein the sheet is reduced to a thickness of less than 0.010 inch during the rolling step. 40
  20. The method of claim 1, wherein the aluminum powder and iron powder each have an average particle size of 10 to 60  $\mu$ m. 45
  21. The method of claim 1, wherein the iron aluminide includes, in weight %, ≤2% Mo, ≤1% Zr, ≤2% Si, ≤30% Ni, ≤10% Cr, ≤0.1% C ≤0.5% Y, ≤0.1% B, ≤1% Nb and ≤1% Ta. 50
  22. The method of claim 1, wherein the iron aluminide consists essentially of, in weight %, 20-32% Al, 0.3-0.5% Mo, 0.05-0.15% Zr, 0.01-0.05% C, ≤25% Al<sub>2</sub>O<sub>3</sub> particles, ≤1% Y<sub>2</sub>O<sub>3</sub> particles, balance Fe. 55
  23. The method of claim 1, wherein the iron aluminide consists essentially of, in weight %, 22-32% Al, 0.3-0.5% Mo, 0.05-0.3% Zr, 0.01-0.1% C, ≤1% Y<sub>2</sub>O<sub>3</sub>, balance Fe. 60
  24. The process of claim 1, wherein the article is formed by cold rolling the mixture with the powder of the mixture in direct contact with rollers of a rolling apparatus. 65
  25. The process of claim 1, wherein the shaping step is carried out by tape casting the powder mixture into a tape or sheet.